

Patented Jan. 22, 1924.

1,481,747

# UNITED STATES PATENT OFFICE.

WILLIAM R. SALTRICK, OF PURLEY, ENGLAND, ASSIGNOR TO ROBERT WICKERSHAM  
STIMSON, OF NEW YORK, N. Y.

## REFINING OF FERROCHROME.

No Drawing.

Application filed January 17, 1923. Serial No. 613,292.

To all whom it may concern:

Be it known that I, WILLIAM ROBERT SALTRICK, a subject of the King of Great Britain, residing at "The Acacias," Higher Drive, Purley, Surrey, England, have invented new and useful Improvements in and Relating to the Refining of Ferrochrome, of which the following is a specification.

The invention relates to the refining of ferro-chrome, whereby the carbon content of the alloy may be reduced or eliminated.

According to the present invention the molten alloy is subjected to a refining blast or blowing operation by means of a gaseous medium containing both oxidizing and reducing gases in the form of steam and hydrogen.

In addition to the use of hydrogen and steam, this gaseous admixture may be used in conjunction with other oxidizing gases, as for example, carbon dioxide and air as oxidizing gases, and carbon monoxide as an additional reducing gas.

This gaseous admixture may be directed on to the surface of the molten alloy, or injected or blown through the molten metal, or the gases may be used for the refining operation in both of these ways.

In carrying out the refining operation according to the present invention, the molten alloy is preferably maintained within a temperature range of 1500° C. to 1600° C., and as near a temperature of 1500° C., as possible. As the refining operation proceeds, a higher temperature may be necessary. But the temperature should not be permitted to rise unduly high, as a lower temperature is more favourable to the production of a refined alloy with a minimum loss of the chromium content. The upper limit of temperature of the molten alloy should not exceed 1650° C., or 1700° C., at the most.

All or part of the steam and hydrogen mixture may be directed so as to impinge on the surface of the molten alloy, in which case extreme fluidity of the alloy may not be so necessary.

I find a convenient way of employing the refining gases so as to work within the desired temperature limits is to impinge a steam and hydrogen mixture on to the surface of the molten alloy and to employ a more vigorous oxidizing gaseous refining admixture for blowing through the molten alloy. This blast through the alloy may be

made more oxidizing in character by means of a proportion of carbon dioxide either with or without air. In this way, the rise of temperature of the alloy by the use of the oxidizing blast blown through the alloy is kept under control by the cooling action of the refining gaseous medium which impinges on the surface.

A convenient form of refining blast within the scope of the invention is producer gas, or water gas, or blast furnace gases, to which a proportion of steam has been added or caused to be included therewith.

As will be understood, the gaseous mixture employed according to my invention may be preheated, in order to avoid too strong a local cooling action at the point where it is projected either through or on to the surface of the molten alloy.

By the use of a blast containing both oxidizing and reducing gases, as in the manner described, the carbon is subjected to an oxidizing action in the well-known manner, while the reducing gas or gases exert a restraining action on the oxidation of the metals of the molten alloy.

I am aware that in the treatment of molten metals such as iron or steel it is known to use a blast of air or steam or both and to dissociate the steam into its constituents but the treatment of ferro-chrome involves considerations peculiar to this alloy. It is well known that this alloy is a difficult alloy to refine economically by reason of its strong affinity for carbon, its high melting point, and its high chromium content.

When the high-carbon molten alloy is refined by treatment with an air blast, as has hitherto been proposed, the oxidation of the carbon and silicon present as impurities rapidly raises the temperature of the molten alloy to a point where severe oxidation of the chromium occurs simultaneously with an elimination of the oxidizable impurities. There is also a loss of chromium by evaporation at the high temperature of the molten bath.

According to the process for the preparation of refined ferro-chrome constituting the present invention, both hydrogen and steam are employed as a refining gaseous mixture and these gases may be used either with or without other suitable gas or gases as has hereinbefore been described. While the steam is both an oxidizing agent and a temperature regulator, and particularly

when used in the manner described, the presence of hydrogen in the refining blast provides for a diminished oxidation of the molten alloy constituents thus permitting the blowing operation to be continued for such a period as will enable the molten alloy to be refined sufficiently without severe losses of the chromium content, which is an important consideration.

10. What I claim is:—

1. A process for refining molten ferro-chrome to produce an alloy of low carbon content, comprising, subjecting molten ferro-chrome to the action of a gaseous mixture containing both hydrogen and steam.
15. 2. A process according to claim 1, the molten ferro-chrome being maintained at a temperature of from 1500° C. to 1650° C.
20. 3. A process for refining molten ferro-chrome to produce an alloy of low carbon

content, comprising, directing a blast of hydrogen and steam to impinge on the surface of a bath of molten ferro-chrome.

4. A process for refining molten ferro-chrome to produce an alloy of low carbon 25 content, comprising, directing blasts of hydrogen and steam both upon the surface of a bath of molten ferro-chrome, and also through the molten mass.

5. A process for refining molten ferro-chrome to produce an alloy of low carbon 30 content, comprising, directing a blast of an oxidizing and reducing gas admixture onto the surface of a bath of molten ferro-chrome, and simultaneously directing a more highly 35 oxidizing gas admixture of oxidizing and reducing gases through the molten ferro-chrome.

W. R. SALTRICK.